



US006881298B2

(12) **United States Patent**  
Rheims et al.

(10) Patent No.: **US 6,881,298 B2**  
(45) Date of Patent: **Apr. 19, 2005**

(54) **PROCESS FOR LOADING FIBERS WITH CALCIUM CARBONATE IN A PLURALITY OF REACTORS**

(75) Inventors: **Jörg Rheims**, Heidenheim (DE); **Klaus Doelle**, Menasha, WI (US); **Oliver Heise**, Menasha, WI (US); **Werner Witek**, Appleton, WI (US)

(73) Assignee: **Voith Paper Patent GmbH**, Heidenheim (DE)

(\*) Notice: Subject to any disclaimer, the term of this patent is extended or adjusted under 35 U.S.C. 154(b) by 14 days.

(21) Appl. No.: **10/369,150**

(22) Filed: **Feb. 19, 2003**

(65) **Prior Publication Data**

US 2003/0121624 A1 Jul. 3, 2003

**Related U.S. Application Data**

(63) Continuation of application No. 09/903,975, filed on Jul. 12, 2001, now Pat. No. 6,599,390.

(30) **Foreign Application Priority Data**

Jul. 13, 2000 (DE) ..... 100 33 978

(51) **Int. Cl.** <sup>7</sup> **D21H 11/16; D21H 17/64**

(52) **U.S. Cl.** ..... **162/9; 162/19; 162/181.2; 162/181.4; 162/182; 162/183**

(58) **Field of Search** ..... **162/9, 181.2, 182, 162/183, 241, 242, 243, 19; 422/188, 194**

(56)

**References Cited**

**U.S. PATENT DOCUMENTS**

|              |          |                       |           |
|--------------|----------|-----------------------|-----------|
| 3,849,247 A  | 11/1974  | Richter .....         | 162/237   |
| 4,431,480 A  | 2/1984   | Markham et al. ....   | 162/19    |
| 4,842,690 A  | 6/1989   | Gazdik et al. ....    | 162/57    |
| 5,096,539 A  | 3/1992   | Allan .....           | 162/9     |
| 5,223,090 A  | 6/1993   | Klungness et al. .... | 162/9     |
| 5,665,205 A  | 9/1997   | Srivatsa et al. ....  | 162/181.4 |
| 5,679,220 A  | 10/1997  | Matthew et al. ....   | 162/181.4 |
| 6,264,794 B1 | 7/2001   | Neumann et al. ....   | 162/205   |
| 6,599,390 B1 | * 7/2003 | Rheims et al. ....    | 162/9     |

**FOREIGN PATENT DOCUMENTS**

|    |             |         |                  |
|----|-------------|---------|------------------|
| EP | 0457235 A1  | 5/1991  | ..... D21H/17/70 |
| EP | 0791685 A2  | 8/1997  | ..... D21H/17/70 |
| GB | 2 265 916 A | 10/1993 | ..... D21H/15/02 |
| WO | WO 97/01670 | 1/1997  | ..... D21H/17/67 |

\* cited by examiner

*Primary Examiner*—Steve Alvo

(74) *Attorney, Agent, or Firm*—Taylor & Aust, P.C.

(57) **ABSTRACT**

For a process and an apparatus for loading fibers contained in a pulp suspension with calcium carbonate, a calcium oxide and/or a medium containing calcium hydroxide is fed to the pulp suspension, and the so treated pulp suspension is further charged in several reactors with pure carbon dioxide or a medium containing carbon dioxide. The reactors can be connected in series and/or in parallel.

**14 Claims, 1 Drawing Sheet**





## 1

**PROCESS FOR LOADING FIBERS WITH  
CALCIUM CARBONATE IN A PLURALITY  
OF REACTORS**

This is a continuation of application Ser. No. 09/903,975 filed Jul. 12, 2001 now U.S. Pat. No. 6,599,390.

**BACKGROUND OF THE INVENTION**

**1. Field of the Invention**

The invention concerns a process for loading fibers contained in a pulp suspension with calcium carbonate.

**2. Description of the Related Art**

Pulp suspensions of the above-mentioned type are used especially in paper and cardboard manufacture. The sparing use of raw material resources, due especially to economical and ecological concerns, is reflected in the paper production industry by the use of paper web with lower basis weights, as well as by the partial replacement of pulp with filling materials. If lower cost raw materials are used, the paper quality should at least be maintained. Among other things, the end product's strength, visual characteristics, and processability play key roles in this challenge.

**SUMMARY OF THE INVENTION**

The present invention relates to a process and apparatus for loading fibers with calcium carbonate, especially in terms of optimum reaction balance, optimum reaction speed and optimum flexibility of production output.

The invention comprises, in one form thereof, a process of fiber loading that includes adding calcium oxide and/or a medium containing calcium hydroxide to a pulp suspension, and then charging the pulp suspension in several reactors with pure carbon dioxide or a medium containing carbon dioxide. Upon the addition of calcium oxide and/or a medium containing calcium hydroxide to the pulp, an exothermic chemical reaction takes place, the calcium hydroxide being added in liquid form (lime milk). By using lime milk, the water settled in or on the pulp suspension's fibrous material is not necessarily required to start and continue the chemical reaction.

Because of this development, the chemical process, which is the basis of the loading, is split into several small processes, thereby permitting an optimum reaction balance, an optimum reaction speed, and an optimum flexibility of production output to be achieved. This use of several small processes enables a targeted and optimal testing of partial reactions, switching on and off of partial reactors and a variation of the operating parameters in the partial reactors.

On loading the fibers, calcium carbonate is imbedded into the wetted fiber surfaces by adding calcium oxide and/or calcium hydroxide to the wet fibrous material. Thereby, at least part of this calcium compound can associate with the water of the pulp mass. The so treated fibrous material is then charged with the pure carbon dioxide or the medium containing carbon dioxide.

As a result, the term "wetted fiber surface" can include all wetted surfaces of the individual fibers. Consequently, the fibers become loaded with calcium carbonate both on their outer surfaces and on their insides (lumen).

Accordingly, the fibers are loaded with the filler material calcium carbonate, whereby the accumulation on the wetted surfaces takes place by a so-called "Fiber Loading™" process, as described in U.S. Pat. No. 5,223,090. In this "Fiber Loading™" process, the carbon dioxide reacts with the calcium hydroxide to form water and calcium carbonate.

## 2

For one suitable arrangement of the process is conformity with the invention, at least one section of the reactor is connected in series. Several smaller reaction volumes are created from one large reaction volume, so that the reaction speed is increased and, correspondingly, the contact surfaces of the reactants are enlarged. Furthermore, in an advantageous manner, (crystallization-) processes can be achieved in a targeted fashion and the parameters for an optimal reaction can be matched.

With a further advantageous arrangement, at least one section of the reactors is connected in parallel. In addition the above-mentioned advantages, this arrangement also allows for optimum adaptability of the production output. It is also of advantage, in parallel-connected reactors, to produce calcium carbonate with different crystal types and, preferably, to mix these on termination of the production process. This mixing allows an optimal composition of the product.

In certain cases, a combination of series- and parallel-connection of the reactors are of benefit. In this way, the parallel section can be matched to the required production range.

In other respects, the loading of fibers with calcium carbonate is as described in U.S. Pat. No. 5,223,090. The content of that patent is hereby incorporated by reference herein.

The apparatus embodying the invention essentially includes several reactors, in which the pulp suspension, mixed with calcium oxide and/or calcium hydroxide, can be charged with pure carbon dioxide or a medium containing carbon dioxide.

**BRIEF DESCRIPTION OF THE DRAWINGS**

The above-mentioned and other features and advantages of this invention, and the manner of attaining them, will become more apparent and the invention will be better understood by reference to the following description of an embodiment of the invention taken in conjunction with the accompanying drawing, wherein:

**40 FIG. 1** is a schematic illustration of an embodiment of the fiber loading apparatus of the present invention.

The exemplification set out herein illustrates one preferred embodiment of the invention, in one form, and such exemplification is not to be construed as limiting the scope of the invention in any manner.

**DETAILED DESCRIPTION OF THE  
INVENTION**

**50 FIG. 1** shows in schematic an apparatus **10** for loading fibers, contained in a pulp suspension, with calcium carbonate ( $\text{CaCO}_3$ ). Correspondingly, apparatus **10** serves to add the calcium carbonate to the wetted fiber surfaces of the fibrous material. In this way, this loading of the fibers, especially in accordance with the aforementioned "Fiber Loading™" process, takes place.

Apparatus **10** includes several reactors **12**, in which the pulp suspension, mixed with calcium oxide ( $\text{CaO}$ ) and/or calcium hydroxide ( $\text{Ca(OH)}_2$ ) can be charged by pure carbon dioxide ( $\text{CO}_2$ ) or by a medium containing carbon dioxide ( $\text{CO}_2$ ). Moreover, reactors **12**, can be connected in series or parallel. It is possible to have a series arrangement, a parallel arrangement, or a combination arrangement of series and parallel for reactors **12**. Also, with parallel-connected reactors **12**, it is possible to produce calcium carbonate with different types of crystal and to mix these, preferably on termination of the respective production process.



## 5

providing a pulp suspension comprised of fibers;  
 providing a calcium-rich medium, said calcium-rich medium being comprised of at least one of calcium oxide and calcium hydroxide;  
 adding controlled amounts of said calcium-rich medium to said pulp suspension and thereby forming a controllably variable calcium-treated pulp suspension;  
 providing a plurality of reactors, each reactor being fluidly coupled to a source of a carbon-dioxide medium, said carbon-dioxide medium being one of pure carbon dioxide and a medium containing carbon dioxide;  
 charging said calcium-treated pulp suspension and said carbon-dioxide medium into a first reactor to promote a chemical reaction to form calcium carbonate and thereby load said fibers with said calcium carbonate;  
 controlling the chemical reaction in the first reactor by selectively adding the carbon dioxide medium in at least one location of upstream, of the first reactor, into the first reactor and downstream of the first reactor, and selectively controlling temperatures of the pulp suspension and the carbon-dioxide medium in at least one location of upstream of the first reactor, in the first reactor and downstream of the first reactor;  
 charging a second reactor with said carbon-dioxide medium and at least one of said calcium-treated pulp suspension and fibers loaded with calcium carbonate from said first reactor; and  
 controlling a chemical reaction in the second reactor to form calcium carbonate with different types of crystals from said calcium carbonate formed in said first reactor, and thereby loading said fibers in said second reactor with said different types of calcium carbonate crystals, including selectively adding the carbon dioxide medium in at least one location of upstream of the second reactor, into the second reactor, and downstream of the second reactor, and selectively controlling temperatures of the pulp suspension and the carbon-dioxide medium in at least one location of upstream of the second reactor, in the second reactor and downstream of the second reactor.

2. The process of claim 1, wherein said plurality of reactors includes at least one section of reactors, said at least one section of reactors being connected in series.

3. The process of claim 1, wherein said plurality of reactors includes at least one section of reactors, said at least one section of reactors being connected in parallel.

4. The process of claim 1, wherein each said reactor has an energy input associated therewith, said energy input being in the approximate range of 0.1 kWh/t to 200 kWh/t.

## 6

5. The process of claim 4, wherein said energy input is in the approximate range of 0.5 kWh/t to 200 kWh/t.

6. The process of claim 1, wherein said plurality of reactors includes a combination of parallel-connected reactors and series-connected reactors.

7. The process of claim 1, wherein each of said pulp suspension and said calcium-treated pulp suspension have a pH associated therewith, the process including the further steps of:

measuring the pH of at least one of said pulp suspension and said calcium-treated pulp suspension so as to thereby monitor the chemical reaction; and

setting the pH of at least one of said pulp suspension and said calcium-treated pulp suspension so as to thereby help control the chemical reaction, the pH thereof being set within a range of about 5.5 to 10.5.

8. The process of claim 1, wherein said pulp suspension has an ash content, said ash content being controllable within an approximate range of 1% to 70%.

9. The process of claim 1, wherein said carbon-dioxide medium is introduced in a gaseous form.

10. The process of claim 1, wherein said carbon-dioxide medium being charged into said at least one reactor has a medium temperature associated therewith, said medium temperature being controlled within an approximate range of -20° C. to 100° C.

11. The process of claim 1, wherein brightness is used as an indicator for controlling the chemical reaction.

12. The process of claim 1, wherein said pulp suspension has an ash content, said pulp suspension and said ash content each having a pH associated therewith, the pH of at least one of said pulp suspension and said ash content being used as a control parameter to at least one of monitor and control the chemical reaction.

13. The process of claim 1, wherein said plurality of reactors includes partial reactors in which partial reactions of calcium-treated pulp suspension and said carbon-dioxide medium have occurred, said process including at least one of the following steps: testing of partial reactions;

switching on and off of at least one partial reactor; and varying at least one operating parameter of at least one partial reactor.

14. The process of claim 1, wherein a pressure associated with each reactor is regulated in the range of about 0.1 bar to about 20 bar.

\* \* \* \* \*